



US005283023A

**United States Patent [19]**

Nohr et al.

[11] **Patent Number:** 5,283,023[45] **Date of Patent:** Feb. 1, 1994[54] **METHOD OF IMPARTING DELAYED WETTABILITY TO A NONWOVEN WEB**[75] Inventors: **Ronald S. Nohr, Roswell; John G. MacDonald, Decatur, both of Ga.**[73] Assignee: **Kimberly-Clark Corporation, Neenah, Wis.**[21] Appl. No.: **818,030**[22] Filed: **Jan. 3, 1992**[51] Int. Cl.<sup>5</sup> ..... **D01F 1/10**[52] U.S. Cl. ..... **264/103; 264/210.6; 264/210.8; 264/211; 264/211.12**[58] Field of Search ..... **264/103, 210.6, 210.8, 264/211, 211.12**[56] **References Cited****U.S. PATENT DOCUMENTS**

|           |         |             |          |
|-----------|---------|-------------|----------|
| 3,016,599 | 1/1962  | Perry       | 428/338  |
| 3,341,394 | 9/1967  | Kinney      | 428/292  |
| 3,655,862 | 4/1972  | Dorschner   | 264/555  |
| 3,692,618 | 9/1972  | Dorschner   | 428/227  |
| 3,704,198 | 11/1972 | Prentice    | 428/198  |
| 3,705,068 | 12/1972 | Dobo        | 156/441  |
| 3,755,527 | 8/1973  | Keller      | 264/518  |
| 3,802,817 | 4/1974  | Matsuki     | 425/66   |
| 3,849,241 | 11/1974 | Butin       | 428/137  |
| 3,853,651 | 12/1974 | Porte       | 156/73.6 |
| 3,978,185 | 8/1976  | Buntin      | 264/518  |
| 4,064,605 | 12/1977 | Akiyama     | 28/100   |
| 4,091,140 | 5/1978  | Harmon      | 428/288  |
| 4,100,319 | 7/1978  | Schwartz    | 428/171  |
| 4,100,324 | 7/1978  | Anderson    | 428/288  |
| 4,118,531 | 10/1978 | Hauser      | 428/224  |
| 4,340,563 | 7/1982  | Appel       | 264/518  |
| 4,405,297 | 9/1983  | Appel       | 425/72.2 |
| 4,434,204 | 2/1984  | Harman      | 428/198  |
| 4,627,811 | 12/1986 | Greiser     | 425/72.2 |
| 4,644,045 | 2/1987  | Fowells     | 526/348  |
| 4,663,220 | 5/1987  | Wisneski    | 428/221  |
| 4,857,251 | 8/1989  | Nohr et al. | 264/103  |
| 4,923,914 | 5/1990  | Nohr        | 524/99   |

**OTHER PUBLICATIONS**

V. A. Wente, "Superfine Thermoplastic Fibers", vol. 48, No. 8, pp. 1342-1346 (1956).

V. A. Wente et al., "Manufacture of Superfine Organic Fibers", NRL Report 4364 (111437), dated May 25, 1954.

Robert R. Butin and Dwight T. Lohkamp, "Melt Blowing—A One-Step Web Process for New Nonwoven Products", vol. 56, No. 4, pp. 74-77 (1973).

*Primary Examiner*—Leo B. Tentoni  
*Attorney, Agent, or Firm*—William E. Maycock[57] **ABSTRACT**

A method of forming a nonwoven web having delayed wettability, in that the web is not wettable by water upon its formation but becomes wettable within from about three hours to about 30 days thereafter without any post-formation treatment, which method involves the steps of (1) melting a mixture consisting of a thermoplastic polyolefin, and additive, and a retardant coadditive; (2) forming fibers by extruding the resulting melt through under defined conditions of shear and throughput; (3) drawing the fibers; and (4) collecting the fibers on a moving foraminous surface as a web of entangled fibers. The additive is a defined polysiloxane polyether having a molecular weight of from about 700 to about 1,300 and a polydispersity of from about 1.3 to about 3.0. The additive is present in an amount of from about 1.8 to about 3.0 percent by weight, based on the amount of thermoplastic polyolefin. The retardant coadditive is a high surface area particulate inorganic or organic material which is insoluble in the polymer at both ambient and melt-extrusion temperatures, is present in an amount of from about 0.1 to about 1 percent, based on the weight of the thermoplastic composition, has a surface area of from about 50 to about 500 m<sup>2</sup>, and is capable of being at least partially coated by the additive.

**7 Claims, No Drawings**

**METHOD OF IMPARTING DELAYED WETTABILITY TO A NONWOVEN WEB**

**CROSS-REFERENCES TO RELATED APPLICATIONS**

The application of the principles of the present invention to nonwoven webs prepared by hydraulic spinning is described and claimed in copending and commonly assigned Application Ser. No. 07/817,267, entitled FILAMENTS, TOW, AND WEBS FORMED BY HYDRAULIC SPINNING AND HAVING DELAYED WETTABILITY and filed of even date in the names of Ronald Sinclair Nohr, Richard Allen Anderson, and John Gavin MacDonald.

The application of the principles of the present invention to nonwoven webs having delayed antimicrobial activity is described and claimed in copending and commonly assigned Application Ser. No. 07/817,271, entitled METHOD OF PREPARING A NONWOVEN WEB HAVING DELAYED ANTIMICROBIAL ACTIVITY and filed of even date in the names of Ronald Sinclair Nohr and John Gavin MacDonald.

The formation of a nonwoven web having delayed wettability is described and claimed in Application Ser. No. 07/566,938, entitled METHOD OF PREPARING A NONWOVEN WEB HAVING DELAYED WETTABILITY and filed on Aug. 13, 1990 in the names of Ronald S. Nohr and J. Gavin MacDonald.

A method of increasing the delay period of the nonwoven webs obtained in Application Ser. No. 07/566,938 is described and claimed in Application Ser. No. 07/488,344, entitled METHOD OF INCREASING THE DELAY PERIOD OF NONWOVEN WEBS HAVING DELAYED WETTABILITY and filed on Mar. 2, 1990 in the names of Ronald S. Nohr and J. Gavin MacDonald, now U.S. Pat. No. 5,114,646.

**BACKGROUND OF THE INVENTION**

The present invention relates to the formation of a nonwoven web by melt extrusion. More particularly, the present invention relates to a method of imparting delayed wettability to a nonwoven web prepared by melt extrusion.

Traditional melt-extrusion processes for the formation of a nonwoven web from a thermoplastic polymer typically involve melting the thermoplastic polymer, extruding the molten polymer through a plurality of orifices to form a plurality of threadlines or filaments, attenuating the filaments by entrainment in a rapidly moving first stream of gas, cooling the filaments with a second stream of gas, and randomly depositing the attenuated filaments, or fibers, on a moving foraminous surface. The most common and well known of these processes are meltblowing, coforming, and spunbonding. The nonwoven webs obtained by these processes are widely used in a variety of products, but especially in such disposable absorbent products as diapers, incontinent products, feminine care products, such as tampons and sanitary napkins, wipes, sterilization wraps, surgical drapes and related materials, hospital gowns, shoe covers, and the like, to name but a few.

Meltblowing references include, by way of example, U.S. Pat. Nos. 3,016,599 to R. W. Perry, Jr., 3,704,198 to J. S. Prentice, 3,755,527 to J. P. Keller et al., 3,849,241 to R. R. Butin et al., 3,978,185 to R. R. Butin et al., and 4,663,220 to T. J. Wisneski et al. See, also, V. A. Wente, "Superfine Thermoplastic Fibers", *Industrial*

and *Engineering Chemistry*, Vol. 48, No. 8, pp. 1342-1346 (1956); V. A. Wente et al., "Manufacture of Superfine Organic Fibers", Navy Research Laboratory, Washington, D.C., NRL Report 4364 (111437), dated May 25, 1954, United States Department of Commerce, Office of Technical Services; and Robert R. Butin and Dwight T. Lohkamp, "Melt Blowing-A One-Step Web Process for New Nonwoven Products", *Journal of the Technical Association of the Pulp and Paper Industry*, Vol. 56, No. 4, pp. 74-77 (1973).

Coforming references (i.e., references disclosing a meltblowing process in which fibers or particles are comingled with the meltblown fibers as they are formed) include U.S. Pat. Nos. 4,100,324 to R. A. Anderson et al. and 4,118,531 to E. R. Hauser.

Finally, spunbonding references include, among others, U.S. Pat. Nos. 3,341,394 to Kinney, 3,655,862 to Dorschner et al., 3,692,618 to Dorschner et al., 3,705,068 to Dobo et al., 3,802,817 to Matsuki et al., 3,853,651 to Porte, 4,064,605 to Akiyama et al., 4,091,140 to Harmon, 4,100,319 to Schwartz, 4,340,563 to Appel and Morman, 4,405,297 to Appel and Morman, 4,434,204 to Hartman et al., 4,627,811 to Greiser and Wagner, and 4,644,045 to Fowells.

The polymers most often used in the foregoing processes, particularly for the types of products mentioned, are polyolefins. These polymers are naturally hydrophobic, which often is an undesirable characteristic.

A significant improvement over previously known methods of imparting hydrophilicity to otherwise hydrophobic polymers is described in U.S. Pat. No. 4,923,914 to Nohr et al., which patent is incorporated herein by reference. The patent describes a surface-segregatable, melt-extrudable thermoplastic composition which comprises at least one thermoplastic polymer and at least one defined additive. The most preferred additives are polysiloxane polyethers.

Upon being melt-extruded, the compositions of U.S. Pat. No. 4,923,914 result in fibers having a differential, increasing concentration of the additive from the centers to the surfaces thereof, such that the concentration of additive toward the surface of each fiber is greater than the average concentration of additive in the more central region of the fiber and imparts to the surface of the fiber at least one desired characteristic which otherwise would not be present. The additive forms an emulsion with the polymer at melt extrusion temperatures, under which conditions the additive and the polymer form a metastable solution. As the temperature of the newly formed fiber drops below melt extrusion temperatures, the additive becomes significantly less compatible with the polymer. Concurrent with this marked change in compatibility, the polymer begins to solidify. Both factors contribute to the rapid migration or segregation of the additive toward the surface which takes place in a controllable manner.

Web integrity sometimes is a problem with the compositions of U.S. Pat. No. 4,923,914. When the additive is a siloxane-containing compound and the desired characteristic is water-wettability, the resulting nonwoven webs can lack integrity upon their formation because of the presence of additive on the surfaces of the fibers. The additive sometimes interferes with the fiber-to-fiber bonding upon which web integrity relies, especially at additive levels of about 1.5 weight percent or higher. In such circumstances, the additive also has a tendency to accumulate over time on the forming wire.

This problem of poor web integrity in nonwoven webs prepared such processes as meltblowing, coforming, and spunbonding can be rectified by instituting process changes. Alternatively, wettability can be delayed as described in Application Ser. No. 07/566,938, entitled METHOD OF PREPARING A NONWOVEN WEB HAVING DELAYED WETTABILITY and filed on Aug. 13, 1990 in the names of Ronald S. Nohr and J. Gavin MacDonald. The delay in wettability results from the use of a trisiloxane polyether having the general formula,



in which:

- (a)  $\text{R}^1$ - $\text{R}^7$  are independently selected monovalent  $\text{C}^1$ - $\text{C}^3$  alkyl groups;
- (b)  $\text{R}^8$  is hydrogen or a monovalent  $\text{C}^1$ - $\text{C}^3$  alkyl group;
- (c)  $m$  represents an integer of from 0 to about 5;
- (d)  $n$  represents an integer of from 3 to about 8;
- (e) the molecular weight is from about 350 to about 700;
- (f) the polydispersity is from about 1.0 to about 1.3; and
- (g) the trisiloxane polyether is present in an amount of from about 0.5 to about 1.75 percent by weight, based on the amount of thermoplastic polymer, which amount, if homogeneously distributed throughout the polyolefin, is not sufficient to render the polyolefin wettable by water.

A method of increasing the wettability delay period of the nonwoven webs obtained in cross-referenced Application Ser. No. 07/566,938 is disclosed in cross-referenced Application Ser. No. 07/488,344. Such increase in the delay period results from including in the thermoplastic composition, in addition to the defined trisiloxane polyether, from about 0.1 to about 6 percent by weight, based on the amount of thermoplastic polymer, of at least one material having the capacity to increase the delay period for up to about two weeks. The preferred material for increasing the delay period is a phthalocyanine dye.

Notwithstanding the teachings of Application Ser. Nos. 07/566,938 and 07/488,344, there still is need for a method of further delaying the development of wettability in nonwoven webs in a more controlled manner. In addition, there is a need to provide greater time control and to extend the wettability delay period. Furthermore, a method is needed which avoids coloring the fibers as with the use of a phthalocyanine dye.

#### SUMMARY OF THE INVENTION

It therefore is an object of the present invention to provide a method of forming a nonwoven web having delayed wettability.

This and other objects will be apparent to those having ordinary skill in the art from a consideration of the specification and claims which follow.

Accordingly, the present invention provides a method of forming a nonwoven web having delayed wettability, in that said web is not wettable by water upon its formation but becomes wettable within from about three hours to about 30 days thereafter without

any post-formation treatment, which method comprises the steps of:

- (A) melting a mixture which comprises a thermoplastic polyolefin, an additive, and a retardant coadditive;
  - (B) forming fibers by extruding the resulting melt through a die at a shear rate of from about 50 to about 30,000  $\text{sec}^{-1}$  and a throughput of no more than about 5.4  $\text{kg}/\text{cm}/\text{hour}$ ;
  - (C) drawing said fibers; and
  - (D) collecting said fibers on a moving foraminous surface as a web of entangled fibers;
- in which:

- (1) said additive has the general formula I,



in which:

- (a)  $\text{R}_1$ - $\text{R}_9$  are independently selected monovalent  $\text{C}^1$ - $\text{C}^3$  alkyl groups;
- (b)  $\text{R}_{10}$  is either hydrogen or a monovalent  $\text{C}^1$ - $\text{C}^3$  alkyl group;
- (c)  $m$  represents an integer of from 1 to 3;
- (d)  $n$  represents an integer of from 0 to about 5;
- (e)  $p$  represents an integer of from 0 to about 5;
- (f)  $x$  represents an integer of from 1 to about 10;
- (g)  $y$  represents an integer of from 0 to about 5;
- (h) the ratio of  $x$  to  $y$  is equal to or greater than 2;
- (i) said additive has a molecular weight of from about 700 to about 1,300;
- (j) said additive has a polydispersity of from about 1.3 to about 3.0; and
- (k) said additive is present in an amount of from about 1.8 to about 3.5 percent by weight, based on the amount of thermoplastic polyolefin;

or the general formula II,



in which:

- (a)  $\text{R}_{11}$  and  $\text{R}_{14}$  independently are either hydrogen or a monovalent  $\text{C}^1$ - $\text{C}^3$  alkyl group;
- (b)  $\text{R}_{12}$  and  $\text{R}_{13}$  are independently selected monovalent  $\text{C}^1$ - $\text{C}^3$  alkyl groups;
- (c)  $q$  represents an integer from about 1 to about 12;
- (d)  $x$  represents an integer from 1 to about 10;
- (e)  $y$  represents an integer from 0 to about 5; and
- (f) the ratio of  $x$  to  $y$  is equal to or greater than 2;
- (g) said additive has a molecular weight of from about 700 to about 1,300;
- (h) said additive has a polydispersity of from about 1.3 to about 3.0; and
- (i) is present in an amount of from about 1.8 to about 3.5 percent by weight, based on the amount of thermoplastic polyolefin; and
- (2) said retardant coadditive is a high surface area particulate inorganic or organic material, which retardant coadditive:

  - (a) is insoluble in the polymer at both ambient and melt-extrusion temperatures;

- (b) is present in an amount of from about 0.1 to about 1 percent, based on the weight of said thermoplastic composition;
- (c) has a surface area of from about 50 to about 1,000  $\text{m}^2$ ; and
- (d) is capable of being at least partially coated by said additive.

In preferred embodiments, the polyolefin is polypropylene. In other preferred embodiments, the additive molecular weight is in the range of from about 750 to 10,000.

The method of the present invention is particularly useful in the manufacture of articles involving the bonding of one or more nonwoven webs to a substrate, including other nonwoven webs, when adhesive performance would be compromised by the presence of a polysiloxane polyether on the surfaces of the fibers of the nonwoven webs. Examples of such articles include, by way of illustration only, such disposable absorbent products as diapers; incontinent products; feminine care products, such as tampons and sanitary napkins; wipes; and the like. 15 20

## DETAILED DESCRIPTION OF THE INVENTION

## Definitions

As used herein, the term "delayed wettability" as applied to a nonwoven web means that the web is not wettable by water upon its formation but becomes wettable thereafter without any post-formation treatment. 30

The term "post-formation treatment" means any process step or treatment of any kind after the fibers have been formed and collected as a nonwoven web on the moving foraminous surface, which process step or treatment is required in order to induce wettability. Thus, in the absence of a post-formation treatment, wettability develops spontaneously after a given period of time. 35

In general, the term "thermoplastic polyolefin" is used herein to mean any thermoplastic polyolefin which can be used for the preparation of nonwoven webs. Examples of thermoplastic polyolefins include polyethylene, polypropylene, poly(1-butene), poly(2-butene), poly(1-pentene), poly(2-pentene), poly(3-methyl-1-pentene), poly(4-methyl-1-pentene), 1,2-poly-1,3-butadiene, 1,4-poly-1,3-butadiene, polyisoprene, polychloroprene, polyacrylonitrile, poly(vinyl acetate), poly(vinylidene chloride), polystyrene, and the like. 40 45

The preferred polyolefins are those which contain only hydrogen and carbon atoms and which are prepared by the addition polymerization of one or more unsaturated monomers. Examples of such polyolefins include, among others, polyethylene, polypropylene, poly(1-butene), poly(2-butene), poly(1-pentene), poly(2-pentene), poly(3-methyl-1-pentene), poly(4-methyl-1-pentene), 1,2-poly-1,3-butadiene, 1,4-poly-1,3-butadiene, polyisoprene, polystyrene, and the like. In addition, such term is meant to include blends of two or more polyolefins and random and block copolymers prepared from two or more different unsaturated monomers. Because of their commercial importance, the most preferred polyolefins are polyethylene and polypropylene.

## ADDITIVE DESCRIPTION

The additive which is employed in the method of the present invention is a polysiloxane polyether having either formula I or formula II.

## ADDITIVE FORMULA I

This additive has the formula,



in which:

- (a)  $R_1$ - $R_9$  are independently selected monovalent  $C_1$ - $C_3$  alkyl groups;
  - (b)  $R_{10}$  is either hydrogen or a monovalent  $C_1$ - $C_3$  alkyl group;
  - (c)  $m$  represents an integer from 1 to 3;
  - (d)  $n$  represents an integer from 0 to about 5;
  - (e)  $p$  represents an integer from 0 to about 5;
  - (f)  $x$  represents an integer from 1 to about 10;
  - (g)  $y$  represents an integer from 0 to about 5; and
  - (h) the ratio of  $x$  to  $y$  is equal to or greater than 2.

In preferred embodiments, each of  $R_1$ - $R_9$  is a methyl group. In other preferred embodiments,  $R_{10}$  is either hydrogen or a methyl group. In yet other preferred embodiments,  $p$  is either 1 or 2,  $x$  is about 8, and  $y$  is 0.

## ADDITIVE FORMULA II

This additive has the formula,



in which:

- (a)  $R_{11}$  and  $R_{14}$  independently are either hydrogen or a monovalent  $C_1$ - $C_3$  alkyl group;
  - (b)  $R_{12}$  and  $R_{13}$  are independently selected monovalent  $C_1$ - $C_3$  alkyl groups;
  - (c)  $q$  represents an integer from about 1 to about 12;
  - (d)  $x$  represents an integer from 1 to about 10;
  - (e)  $y$  represents an integer from 0 to about 5; and
  - (f) the ratio of  $x$  to  $y$  is equal to or greater than 2.

In preferred embodiments, each of  $R_{12}$ - $R_{13}$  is a methyl group. In other preferred embodiments, each of  $R_{11}$  and  $R_{14}$  independently is either hydrogen or a methyl group. In yet other preferred embodiments,  $x$  is about 8, and  $y$  is 0.

## GENERAL ADDITIVE REQUIREMENTS

While the additive molecular weight can vary from about 700 to about 1,300, it preferably will be in the range of from about 750 to about 1,000.

As noted, the polydispersity of the additive will be in the range of from about 1.3 to about 3.0. As used herein, the term "polydispersity" refers to the ratio of the weight-average molecular weight to the number-average molecular weight. Preferably, the polydispersity of the additive will be in the range of from 1.3 to about 1.8. More preferably, the polydispersity of the additive will be about 1.5.

While the additive can be either a liquid or a solid, a liquid is preferred. It also is preferred that a liquid additive have a surface tension which is less than that of virgin polymer.

In general, the additive will be present in an amount of from about 1.8 to about 3.5 percent by weight, based

on the amount of thermoplastic polyolefin. Preferably, the amount of additive will be in the range of from about 2 to about 2.5 percent by weight. These additive levels are not sufficient to impart hydrophilicity to the polyolefin if the additive is distributed homogeneously or uniformly throughout the polymer. If additive levels greater than about 3.5 percent by weight are employed, the resulting fibers are immediately wettable and the web integrity and deposition problems mentioned earlier often are observed.

It may be noted at this point that optimum additive levels are in part dependent upon the nonwoven process employed. For example, if a given additive were employed at the same level in both a meltblowing process and a spunbonding process, the delay time for the meltblown web is likely to be longer than that for the spunbonded web. Thus, in general, preferred additive levels for meltblowing processes typically are a higher than the preferred additive levels for spunbonding processes. Stated differently, in order to achieve a delay period in a meltblowing processes which is the same as that for a spunbonded process, the level of additive employed in the meltblowing process must be increased. Such increase typically will be of the order of about 0.5 percent.

The term "additive" is used broadly herein to encompass the use of more than one additive in a given composition, i.e., a mixture of two or more additives. Moreover, it should be appreciated by those having ordinary skill in the art that additives as defined herein typically are not available as pure compounds. Thus, the presence of impurities or related materials which may not come within the general formula given above for the additives does remove any given material from the spirit and scope of the present invention. For example, the preparation of additives useful in the present invention typically results in the presence of free polyether. The presence of such free polyether is not known to have deleterious effects, although, in order to achieve a desired delay time with a given additive, it may be necessary to increase the amount of additive to compensate for the presence of free polyether. As a practical matter, it is preferred that the amount of free polyether present in any additive be no more than about 30 percent by weight. More preferably, the amount of free polyether present in an additive will be no more than about 20 percent by weight.

#### RETARDANT COADDITIVE DESCRIPTION

In addition to the additive, the thermoplastic polyolefin to be melt-processed to form a nonwoven web must include a retardant coadditive which is a high surface area particulate inorganic or organic material, which retardant coadditive (a) is insoluble in the polymer at both ambient and melt-extrusion temperatures; (b) is present in an amount of from about 0.1 to about 1 percent, based on the weight of said thermoplastic composition; (c) has a surface area of from about 50 to about 1,000 m<sup>2</sup>, and (d) is capable of being at least partially coated by said additive. Such retardant coadditive preferably will be present in the thermoplastic composition at a level of from about 0.3 to about 0.7 percent by weight.

The retardant coadditive can be any inorganic or organic material having the requisite surface area. In addition, the retardant coadditive must be stable under melt-extrusion conditions. Moreover, the retardant coadditive must be capable of being at least partially

coated by the additive. Stated differently, the additive must have a surface tension which is less than the surface free energy of the retardant coadditive particles.

In general, the shear rate required by the method of the present invention will be in the range of from about 50 to about 30,000 sec<sup>-1</sup>. Preferably, the shear rate will be in the range of from about 150 to about 5,000 sec<sup>-1</sup>, and most preferably from about 300 to about 2,000 sec<sup>-1</sup>.

10 Throughput is of importance because it affects the time the newly formed fiber or film is in a sufficiently molten or fluid state to allow migration or segregation of the additive toward the newly formed surfaces, even though throughput also affects the shear rate.

15 Throughput typically will be in the range of from about 0.01 to about 5.4 kg/cm/hour. Preferably, throughput will be in the range from about 0.1 to about 4.0 kg/cm/hour. The throughput most preferably will be in the range of from about 0.5 to about 2.5 kg/cm/hour.

20 Without wishing to be bound by theory, it is believed that the polysiloxane polyether additives emulsify readily in a polyolefin such as polypropylene to form micelle structures or aggregates. However, silicone polyether additives with molecular weights below 25 about 1,400 form thermally unstable aggregates. That is, the lower the molecular weight of the polysiloxane polyether additive, the more thermally unstable are the micelle structures. At fiber process conditions at temperatures above about 170° C., such additives with molecular weights of around 600-700 readily "break apart" from their poorly packed aggregate structures. The additives then are able to diffuse to the newly forming fiber surfaces.

30 35 However, the lower molecular weight components, in the total molecular weight distribution, not only break apart more readily from their micelle structures at temperature above about 170° C., but they also are capable of diffusing more rapidly than the higher molecular weight species. Thus, the molecular weight distribution or polydispersity requirement is central to the present invention. That is, it is essential that the additive have a relatively high polydispersity in order to minimize the amounts of lower molecular weight components.

In other words, broad molecular weight dispersions contain molecular species that will migrate to the fiber surfaces long after the fibers have been formed. In order to avoid spontaneous surface segregation of low molecular weight species, larger concentrations of higher molecular weight species are required. Segregation control and to some extent, synthetic realities, require broad molecular weight dispersions or polydispersities in concert with higher additive concentrations.

50 55 60 While the polysiloxane polyether additive still tends to migrate to the surfaces of the fibers, the rate of migration is slower because the higher molecular weight components diffuse more slowly than the lower molecular weight components. Moreover, the diffusion or migration of all components of the additive are delayed by the retardant coadditive. It is believed that the delay results from a temporary affinity of the additive for the surfaces of the retardant coadditive particles. Consequently, the retardant coadditive must have a relatively high surface area in order to affect essentially all of the additive. Hence, the additive, additive molecular weight, additive polydispersity, additive concentration, retardant coadditive, and retardant coadditive concen-

tration can be selected so as to give a predetermined delay time.

Having thus described the invention, numerous changes and modifications thereof will be readily apparent to those having ordinary skill in the art without departing from the spirit or scope of the invention.

What is claimed is:

1. A method of forming a nonwoven web having delayed wettability, in that said web is not wettable by water upon its formation but becomes wettable within 10 from about three hours to about 30 days thereafter without any post-formation treatment, which method comprises the steps of:

(A) melting a mixture which comprises a thermoplastic polyolefin, an additive, and a retardant coadditive; 15

(B) forming fibers by extruding the resulting melt through a die at a shear rate of from about 50 to about 30,000 sec<sup>-1</sup> and a throughput of no more than about 5.4 kg/cm/hour; 20

(C) drawing said fibers; and

(D) collecting said fibers on a moving foraminous surface as a web of entangled fibers;

in which:

(1) said additive has the general formula I, 25



in which:

(a) R<sub>1</sub>-R<sub>9</sub> are independently selected monovalent 35 C<sub>1</sub>-C<sub>3</sub> alkyl groups;

(b) R<sub>10</sub> is either hydrogen or a monovalent C<sub>1</sub>-C<sub>3</sub> alkyl group;

(c) m represents an integer of from 1 to 3;

(d) n represents an integer of from 0 to about 5;

(e) p represents an integer of from 0 to about 5;

(f) x represents an integer of from 1 to about 10;

(g) y represents an integer of from 0 to about 5;

(h) the ratio of x to y is equal to or greater than 2;

(i) said additive has a molecular weight of from 45 about 700 to about 1,300;

(j) said additive has a polydispersity of from about 1.3 to about 3.0; and

(k) said additive is present in an amount of from 50 about 1.8 to about 3.0 percent by weight, based on the amount of thermoplastic polyolefin;

or the general formula II,



in which:

(a) R<sub>11</sub> and R<sub>14</sub> independently are either hydrogen or a monovalent C<sub>1</sub>-C<sub>3</sub> alkyl group;

(b) R<sub>12</sub> and R<sub>13</sub> are independently selected monovalent C<sub>1</sub>-C<sub>3</sub> alkyl groups;

(c) q represents an integer from about 1 to about 12;

(d) x represents an integer from 1 to about 10;

(e) y represents an integer from 0 to about 5; and

(f) the ratio of x to y is equal to or greater than 2;

(g) said additive has a molecular weight of from about 700 to about 1,300;

(h) said additive has a polydispersity of from about 1.3 to about 3.0; and

(i) is present in an amount of from about 1.8 to about 3.5 percent by weight, based on the amount of thermoplastic polyolefin; and

(2) said retardant coadditive is a high surface area particulate inorganic or organic material, which retardant coadditive:

(a) is insoluble in the polymer at both ambient and meltextrusion temperatures;

(b) is present in an amount of from about 0.1 to about 1 percent, based on the weight of said thermoplastic composition;

(c) has a surface area of from about 50 to about 1,000 m<sup>2</sup>; and

(d) is capable of being at least partially coated by said additive.

2. The method of claim 1, in which said polyolefin is polypropylene.

3. The method of claim 1, in which said additive has a molecular weight of from about 750 to about 1,000.

4. The method of claim 1, in which said additive is present in an amount of from about 2.0 to about 2.5 percent by weight, based on the amount of thermoplastic polymer.

5. The method of claim 1, in which the shear rate is from about 150 to about 5,000 sec<sup>-1</sup>.

6. The method of claim 1, in which the throughput is in the range of from about 0.1 to about 4.0 kg/cm/hour.

7. The method of claim 1, in which the additive, additive molecular weight, additive polydispersity, additive concentration, retardant coadditive, and retardant coadditive concentration are selected so as to give a predetermined delay time.

\* \* \* \* \*